



US012365963B2

(12) **United States Patent**  
**Laws et al.**

(10) **Patent No.:** US 12,365,963 B2  
(45) **Date of Patent:** Jul. 22, 2025

(54) **COPPER ALLOYS**

(71) Applicant: **ADVANCED ALLOY HOLDINGS PTY LTD**, Freshwater (AU)

(72) Inventors: **Kevin James Laws**, Freshwater (AU); **Peter Tyrrell Nicholson**, Freshwater (AU); **Patrick Lars Joseph Conway**, Freshwater (AU); **Lori Cheryl Bassman**, Freshwater (AU); **Warren Richard McKenzie**, Freshwater (AU)

(73) Assignee: **ADVANCED ALLOY HOLDINGS PTY LTD**, Freshwater (AU)

(\*) Notice: Subject to any disclaimer, the term of this patent is extended or adjusted under 35 U.S.C. 154(b) by 0 days.

(21) Appl. No.: **17/765,490**

(22) PCT Filed: **Oct. 2, 2020**

(86) PCT No.: **PCT/AU2020/051062**

§ 371 (c)(1),

(2) Date: **Mar. 31, 2022**

(87) PCT Pub. No.: **WO2021/062485**

PCT Pub. Date: **Apr. 8, 2021**

(65) **Prior Publication Data**

US 2022/0372596 A1 Nov. 24, 2022

(30) **Foreign Application Priority Data**

Oct. 3, 2019 (AU) ..... 2019903725

(51) **Int. Cl.**

**C22C 9/05** (2006.01)

**C22C 30/02** (2006.01)

**C22C 30/06** (2006.01)

(52) **U.S. Cl.**

CPC ..... **C22C 9/05** (2013.01); **C22C 30/02** (2013.01); **C22C 30/06** (2013.01)

(58) **Field of Classification Search**

None

See application file for complete search history.

(56) **References Cited**

U.S. PATENT DOCUMENTS

4,525,434 A \* 6/1985 Morikawa ..... C22C 9/04  
428/929

4,587,097 A 5/1986 Rabinkin et al.  
(Continued)

FOREIGN PATENT DOCUMENTS

CN 1948531 4/2007  
CN 1948531 A \* 4/2007  
(Continued)

OTHER PUBLICATIONS

English language machine translation of CN-1948531-A to Guo.  
Generated Feb. 23, 2023. (Year: 2023).\*  
(Continued)

Primary Examiner — Brian D Walck

(74) Attorney, Agent, or Firm — NORTON ROSE  
FULBRIGHT US LLP

(57) **ABSTRACT**

An alloy comprising or consisting of 40 to 62.5 atomic percent copper, 5 to 40 atomic percent manganese, up to 24 atomic percent nickel, 5 to 24 atomic percent zinc, and 1 to 15 atomic percent aluminium.

17 Claims, 3 Drawing Sheets



(56)

## References Cited

## U.S. PATENT DOCUMENTS

- 2011/0165013 A1\* 7/2011 Trybus ..... C22C 9/01  
420/479
- 2013/0140066 A1 6/2013 Okuno et al.
- 2017/0349975 A1\* 12/2017 Laws ..... C22F 1/16

## FOREIGN PATENT DOCUMENTS

- |    |              |           |
|----|--------------|-----------|
| CN | 101012522    | 8/2007    |
| CN | 109385610    | 2/2019    |
| DE | 102012014851 | 3/2013    |
| GB | 1272737      | 5/1972    |
| JP | 55141540 A   | * 11/1980 |
| JP | S 55141540   | 11/1980   |
| JP | 59-52223     | 12/1984   |
| JP | 2013120411   | 6/2013    |

## OTHER PUBLICATIONS

- English language machine translation of JP-55141540-A. Generated May 3, 2024. (Year: 2024).\*
- International Search Report and Written Opinion issued in Corresponding PCT Application No. PCT/AU2020/051062, dated Nov. 25, 2020.
- Kansky et al., "Quaternary Diffusion in the Cu—Ni—Zn—Mn System at 775° C." *Metallurgical Transactions A*, 1985, vol. 16A, pp. 1123-1132 p. 1124, table 1.
- Office Action issued in corresponding CN Application No. CN 202080076604.8, dated Feb. 18, 2023. (English Translation Provided).
- Office Action Supplement issued in corresponding CN Application No. CN 202080076604.8. (English Translation Provided).
- Extended European Search Report issued in corresponding EP Application No. EP 20872396.5, dated Apr. 4, 2023.
- Masaki Morikawa, *Piping Engineering*, vol. 27, Issue 4, pp. 112-114, 131.
- Wu X. X. et al., "Effect of stacking fault energy on mechanical behavior of cold-forging Cu and Cu alloys," *Materials and Design* 47 (2013) 372-376.
- Ritchie R. O., "The conflicts between strength and toughness," *Nature Materials*, vol. 10, Nov. 2011, pp. 817-822.

Laws K. J. et al., "High entropy brasses and bronzes—Microstructure, phase evolution, and properties," *Journal of Alloys and Compounds* 650 (2015) 949-961.

Campbell F.C., ed., "Phase Diagrams—Understanding the Basics," ASM International, 2012, Ch1:pp. 1-9; 11.

Hillert M., "Phase Equilibria, Phase Diagrams and Phase Transformations," Cambridge University Press, New York, 2nd Edition, 2008, pp. 75-76; 166; 365-367.

Mittemeier E. J., "Fundamentals of Materials Science; The Microstructure—Property Relationship Using Metals as Model Systems," 2nd Ed. Pub:Springer Nature Switzerland AG 2011, 2021, pp. 100-103; 148-169; 365-398; 688-690.

Hull D. and Bacon D. J., "Introduction to Dislocations," 5<sup>th</sup> Edition, Pub: Butterworth-Heinemann 2011; pp. 85-93 and 232-245.

Li Z. et al., "Mechanical properties of high-entropy alloys with emphasis on face-centered cubic alloys," *Progress in Materials Science* 2019, 102, pp. 296-345.

Okamoto H., Schlesinger M.E., and Mueller E.M., Eds., "Cu (Copper) Binary Alloy Phase Diagrams," ASM Handbook, vol. 3: Alloy Phase Diagrams, Pub: ASM International 2016, pp. 304-326.

Davis J.R., "Copper and Copper Alloys," Pub: ASM International, 2001, pp. 7; 39-45; 267.

Sun W. et al., "Experimental investigation and thermodynamic modelling of the Cu—Mn—Ni system," *CALPHAD: Computer Coupling of Phase Diagrams and Thermochemistry* 33 (2009) 642-649.

Alan Prince, K.C. Hari Kumar and MSIT ® (2004) G. Effenberg (ed.) MSI Eureka in SpringerMaterials "Al—Cu—Ni Ternary Phase Diagram Evaluation", 38 pages.

D. Matusch, J. Gröbner, V. Turkevich and MSIT ® (2006) G. Effenberg (ed.) MSI Eureka in SpringerMaterials "Cu—Mn—Zn Ternary Phase Diagram Evaluation," 18 pages.

G. Ghosh and J. Van Humbeeck, P. Perrot and MSIT ® (2004) G. Effenberg (ed.) MSI Eureka in SpringerMaterials "Al—Cu—Zn Ternary Phase Diagram Evaluation," 36 pages.

An X.H. et al., "The influence of stacking fault energy on the mechanical properties of nanostructured Cu and Cu—Al alloys processed by high-pressure torsion," *Scripta Materialia*, vol. 64, 2011, pp. 954-957.

Zhao Y.H. et al., "Evolution of defect structures during cold rolling of ultrafine-grained Cu and Cu—Zn alloys: Influence of stacking fault energy," *Materials Science and Engineering: A*, vol. 474, 2008 pp. 342-347.

\* cited by examiner

**FIGURE 1**



FIGURE 2



**FIGURE 3**



**FIGURE 4**

# 1

## COPPER ALLOYS

### CROSS-REFERENCE TO RELATED APPLICATIONS

This application is a national phase application under 35 U.S.C. § 371 of International Application No. PCT/AU2020/051062, filed Oct. 2, 2020, which claims priority to and the benefit of Australian Application No. 2019903725, filed Oct. 3, 2019. The contents of the aforementioned patent applications are incorporated into the present application by reference.

### FIELD OF THE DISCLOSURE

The present invention relates generally to alloys, and in particular, to copper alloys.

### BACKGROUND OF THE DISCLOSURE

Any discussion of the prior art throughout this specification should in no way be considered as an admission that such prior art is widely known or forms part of the common general knowledge in the field.

Copper-nickel alloys have a range of uses including in heat extractors and radiators where good thermal conductivity is desirable, and in marine settings where corrosion resistance is desirable. However, such alloys can be expensive to manufacture and difficult to work. In this context, there is a need for new alloys having improved mechanical properties. It would also be advantageous to reduce certain costs associated with manufacturing alloys.

### SUMMARY OF THE DISCLOSURE

In a first aspect, the present disclosure provides an alloy comprising or consisting of: 40 to 62.5 atomic percent copper; 5 to 40 atomic percent manganese; up to 24 atomic percent nickel; 5 to 24 atomic percent zinc; and 1 to 15 atomic percent aluminium.

In some examples, the alloy comprises or consists of: 40 to 62.5 atomic percent copper; 5 to 40 atomic percent manganese; 1 to 24 atomic percent nickel; 5 to 24 atomic percent zinc; and 1 to 15 atomic percent aluminium.

In some examples, the alloy comprises or consists of: 40 to 62.5 atomic percent copper; 8 to 40 atomic percent manganese; 1 to 24 atomic percent nickel; 5 to 24 atomic percent zinc; and 1 to 15 atomic percent aluminium.

In some examples, the alloy comprises or consists of: 40 to 62.5 atomic percent copper; 8 to 40 atomic percent manganese; 1 to 8 atomic percent nickel; 5 to 24 atomic percent zinc; and 1 to 15 atomic percent aluminium.

In some examples, the alloy comprises or consists of: 40 to 62.5 atomic percent copper; 8 to 40 atomic percent manganese; 1 to 8 atomic percent nickel; 5 to 24 atomic percent zinc; and 1 to 8 atomic percent aluminium.

In some examples, the alloy comprises or consists of: 40 to 62.5 atomic percent copper; 8 to 40 atomic percent manganese; 1 to 8 atomic percent nickel; 5 to 24 atomic percent zinc; and 1 to 5 atomic percent aluminium.

In some examples, the alloy comprises or consists of: 45 to 62.5 atomic percent copper; 8 to 40 atomic percent manganese; 1 to 8 atomic percent nickel; 5 to 24 atomic percent zinc; and 1 to 5 atomic percent aluminium.

In some examples, the alloy comprises or consists of: 45 to 60 atomic percent copper; 8 to 40 atomic percent man-

# 2

ganese; 1 to 8 atomic percent nickel; 5 to 24 atomic percent zinc; and 1 to 5 atomic percent aluminium.

In some examples, the alloy comprises or consists of: 45 to 60 atomic percent copper; 12.5 to 40 atomic percent manganese; 1 to 8 atomic percent nickel; 5 to 24 atomic percent zinc; and 1 to 5 atomic percent aluminium.

In some examples, the alloy comprises or consists of: 45 to 60 atomic percent copper; 12.5 to 35 atomic percent manganese; 1 to 8 atomic percent nickel; 5 to 24 atomic percent zinc; and 1 to 5 atomic percent aluminium.

In some examples, the alloy comprises or consists of: 45 to 60 atomic percent copper; 12.5 to 35 atomic percent manganese; 1 to 7 atomic percent nickel; 5 to 24 atomic percent zinc; and 1 to 5 atomic percent aluminium.

In some examples, the alloy comprises or consists of: 45 to 60 atomic percent copper; 12.5 to 35 atomic percent manganese; 1 to 7 atomic percent nickel; 7.5 to 24 atomic percent zinc; and 1 to 5 atomic percent aluminium.

In some examples, the alloy comprises or consists of: 45 to 60 atomic percent copper; 12.5 to 35 atomic percent manganese; 1 to 7 atomic percent nickel; 7.5 to 20 atomic percent zinc; and 1 to 5 atomic percent aluminium.

In some examples, the alloy comprises or consists of: 45 to 60 atomic percent copper; 12.5 to 35 atomic percent manganese; 3 to 5 atomic percent nickel; 12.5 to 20 atomic percent zinc; and 1 to 3 atomic percent aluminium.

In some examples, the alloy comprises or consists of: 50 to 60 atomic percent copper; 12.5 to 35 atomic percent manganese; 1 to 7 atomic percent nickel; 7.5 to 20 atomic percent zinc; and 1 to 5 atomic percent aluminium.

In some examples, the alloy comprises or consists of: 50 to 60 atomic percent copper; 15 to 35 atomic percent manganese; 1 to 7 atomic percent nickel; 7.5 to 20 atomic percent zinc; and 1 to 5 atomic percent aluminium.

In some examples, the alloy comprises or consists of: 50 to 60 atomic percent copper; 15 to 22.5 atomic percent manganese; 1 to 7 atomic percent nickel; 7.5 to 20 atomic percent zinc; and 1 to 5 atomic percent aluminium.

In some examples, the alloy comprises or consists of: 50 to 60 atomic percent copper; 15 to 22.5 atomic percent manganese; 1 to 5 atomic percent nickel; 7.5 to 20 atomic percent zinc; and 1 to 5 atomic percent aluminium.

In some examples, the alloy comprises or consists of: 50 to 60 atomic percent copper; 15 to 22.5 atomic percent manganese; 1 to 5 atomic percent nickel; 15 to 20 atomic percent zinc; and 1 to 5 atomic percent aluminium.

In some examples, the alloy comprises or consists of: 50 to 60 atomic percent copper; 15 to 22.5 atomic percent manganese; 1 to 5 atomic percent nickel; 15 to 20 atomic percent zinc; and 1 to 3 atomic percent aluminium.

In some examples, the alloy comprises or consists of: 50 to 60 atomic percent copper; 22.5 to 35 atomic percent manganese; 1 to 5 atomic percent nickel; 5 to 12.5 atomic percent zinc; and 1 to 3 atomic percent aluminium.

In some examples, the alloy comprises or consists of: 40 to 62.5 atomic percent copper; 17 to 35 atomic percent manganese; 1 to 7 atomic percent nickel; 10 to 24 atomic percent zinc; and 1 to 5 atomic percent aluminium.

In some examples, the alloy comprises or consists of: 45 to 60 atomic percent copper; 17 to 35 atomic percent manganese; 1 to 5 atomic percent nickel; 10 to 20 atomic percent zinc; and 1 to 5 atomic percent aluminium.

In some examples, the alloy comprises or consists of: 50 to 60 atomic percent copper; 17 to 35 atomic percent manganese; 1 to 5 atomic percent nickel; 10 to 20 atomic percent zinc; and 1 to 5 atomic percent aluminium.

In some examples,  $(3 \times \text{atomic percent of aluminium}) + \text{atomic percent of zinc} + (0.2 \times \text{atomic percent of manganese})$  is between 22.5% and 32.5%.

In some examples, the atomic percent ratio of copper: nickel is at least 9.

In some examples, the alloy has a tensile strain to failure of between about 40% and 65%.

In some examples, the alloy has an ultimate tensile strength of between about 390 MPa and 575 MPa.

In some examples, the alloy has an as-cast hardness ( $H_V$ ) of between about 80 and 170.

In a second aspect, the present disclosure provides an alloy comprising or consisting of: 40 to 62.5 atomic percent copper; 5 to 40 atomic percent manganese; up to 24 atomic percent nickel; 5 to 24 atomic percent zinc; 1 to 15 atomic percent aluminium; up to 20 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony.

In some examples, the alloy comprises or consists of: 40 to 62.5 atomic percent copper; 5 to 40 atomic percent manganese; up to 24 atomic percent nickel; 5 to 24 atomic percent zinc; 1 to 15 atomic percent aluminium; up to 12 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony.

In some examples, the alloy comprises or consists of: 40 to 62.5 atomic percent copper; 5 to 40 atomic percent manganese; up to 24 atomic percent nickel; 5 to 24 atomic percent zinc; 1 to 15 atomic percent aluminium; up to 12 atomic percent of one or more elements selected from the group consisting of arsenic, phosphorus, sulphur and antimony.

In some examples, the alloy comprises or consists of: 40 to 62.5 atomic percent copper; 5 to 40 atomic percent manganese; up to 24 atomic percent nickel; 5 to 24 atomic percent zinc; 1 to 15 atomic percent aluminium; up to 7 atomic percent chromium; up to 8 atomic percent lead; up to 8 atomic percent bismuth; up to 8 atomic percent cobalt; up to 12 atomic percent iron; up to 8 atomic percent carbon; up to 8 atomic percent tin; up to 8 atomic percent silicon; up to 2 atomic percent magnesium; up to 0.5 atomic percent arsenic; up to 0.5 atomic percent phosphorus; up to 0.5 atomic percent sulphur; and up to 0.5 atomic percent antimony.

In some examples, the alloy comprises or consists of: 40 to 62.5 atomic percent copper; 5 to 40 atomic percent manganese; up to 24 atomic percent nickel; 5 to 24 atomic percent zinc; 1 to 15 atomic percent aluminium; up to 5 atomic percent chromium; up to 5 atomic percent lead; up to 2 atomic percent bismuth; up to 8 atomic percent cobalt; up to 12 atomic percent iron; up to 4 atomic percent carbon; up to 2 atomic percent tin; up to 8 atomic percent silicon; up to 2 atomic percent magnesium; up to 0.3 atomic percent arsenic; up to 0.3 atomic percent phosphorus; up to 0.3 atomic percent sulphur; and up to 0.3 atomic percent antimony.

In some examples, the alloy comprises or consists of: 85 to 95 atomic percent copper, manganese, nickel, zinc and aluminium; and balance of one or more elements selected from the group consisting of chromium, lead, bismuth, cobalt, iron, carbon, tin and silicon.

In some examples, the alloy comprises or consists of: 40 to 62.5 atomic percent copper; 17 to 35 atomic percent manganese; 1 to 7 atomic percent nickel; 10 to 24 atomic percent zinc; 1 to 5 atomic percent aluminium; up to 20 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony.

In some examples, the alloy comprises or consists of: 45 to 60 atomic percent copper; 17 to 35 atomic percent manganese; 1 to 5 atomic percent nickel; 10 to 20 atomic percent zinc; 1 to 5 atomic percent aluminium; up to 20 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony.

In some examples, the alloy comprises or consists of: 50 to 60 atomic percent copper; 17 to 35 atomic percent manganese; 1 to 5 atomic percent nickel; 10 to 20 atomic percent zinc; 1 to 5 atomic percent aluminium; up to 20 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony.

In some examples,  $(3 \times \text{atomic percent of aluminium}) + \text{atomic percent of zinc} + (0.2 \times \text{atomic percent of manganese})$  is between 22.5% and 32.5%.

In some examples, the atomic percent ratio of copper: nickel is at least 9.

In some examples, the alloy has a tensile strain to failure of between about 30% and 65%.

In some examples, the alloy has an ultimate tensile strength of between about 390 MPa and 575 MPa.

In some examples, the alloy has an as-cast hardness ( $H_V$ ) of between about 80 and 170.

#### BRIEF DESCRIPTION OF THE DRAWINGS

FIG. 1. Engineering stress/strain curves of alloy samples in tension.

FIG. 2. Engineering stress/strain curves of alloy samples in tension.

FIG. 3. Side profile of Cu—Ni—Mn—Zn—Al tensile specimen fractures. From left to right:  $\text{Cu}_{60}\text{Ni}_5\text{Mn}_{15}\text{Zn}_{17.5}\text{Al}_{2.5}$ ,  $\text{Cu}_{60}\text{Ni}_5\text{Mn}_{12.5}\text{Zn}_{20}\text{Al}_{2.5}$ ,  $\text{Cu}_{57.5}\text{Ni}_5\text{Mn}_{17.5}\text{Zn}_{17.5}\text{Al}_{2.5}$ ,  $\text{Cu}_{57.5}\text{Ni}_5\text{Mn}_{15}\text{Zn}_{20}\text{Al}_{2.5}$ ,  $\text{Cu}_{55}\text{Ni}_5\text{Mn}_{20}\text{Zn}_{17.5}\text{Al}_{2.5}$ ,  $\text{Cu}_{55}\text{Ni}_5\text{Mn}_{17.5}\text{Zn}_{20}\text{Al}_{2.5}$ ,  $\text{Cu}_{52.5}\text{Ni}_5\text{Mn}_{22.5}\text{Zn}_{17.5}\text{Al}_{2.5}$ , and  $\text{Cu}_{52.5}\text{Ni}_5\text{Mn}_{20}\text{Zn}_{20}\text{Al}_{2.5}$ .

FIG. 4. Side profile of Cu—Ni—Mn—Zn—Al tensile specimen fractures. From left to right:  $\text{Cu}_{45}\text{Ni}_5\text{Mn}_{32.5}\text{Zn}_{15}\text{Al}_{2.5}$ ,  $\text{Cu}_{45}\text{Ni}_5\text{Mn}_{35}\text{Zn}_{12.5}\text{Al}_{2.5}$ ,  $\text{Cu}_{47.5}\text{Ni}_5\text{Mn}_{30}\text{Zn}_{15}\text{Al}_{2.5}$ ,  $\text{Cu}_{47.5}\text{Ni}_5\text{Mn}_{32.5}\text{Zn}_{12.5}\text{Al}_{2.5}$ ,  $\text{Cu}_{50}\text{Ni}_5\text{Mn}_{27.5}\text{Zn}_{15}\text{Al}_{2.5}$ ,  $\text{Cu}_{50}\text{Ni}_5\text{Mn}_{30}\text{Zn}_{12.5}\text{Al}_{2.5}$ ,  $\text{Cu}_{52.5}\text{Ni}_5\text{Mn}_{27.5}\text{Zn}_{12.5}\text{Al}_{2.5}$ , and  $\text{Cu}_{52.5}\text{Ni}_5\text{Mn}_{25}\text{Zn}_{15}\text{Al}_{2.5}$ .

#### DETAILED DESCRIPTION

The term "about" is understood to refer to a range of  $\pm 10\%$ , preferably  $\pm 5\%$  or  $\pm 1\%$  or, more preferably,  $\pm 0.1\%$ .

Throughout this specification, unless the context requires otherwise, the word "comprise", or variations such as "comprises" or "comprising" will be understood to imply the inclusion of a stated element, integer or step, or group of elements, integers or steps, but not the exclusion of any other element, integer or step, or group of elements, integers or steps. Thus, in the context of this specification, the term "comprising" means "including principally, but not necessarily solely".

Any numerical range recited herein is intended to include all sub-ranges of the same numerical precision subsumed within the recited range. For example, a range of 1.0 to 5.0 is intended to include all sub-ranges between (and including) the recited minimum value of 1.0 and the recited maximum value of 5.0, that is, having a minimum value equal to or greater than 1.0 and a maximum value equal to or less than 5.0, such as 2.1 to 4.5. Any maximum numerical limitation recited herein is intended to include all lower numerical limitations subsumed therein and any minimum numerical limitation recited herein is intended to include all higher numerical limitations subsumed therein.

The present disclosure provides alloys comprising or consisting of 40 to 62.5 atomic percent copper; 5 to 40 atomic percent manganese; up to 24 atomic percent nickel; 5 to 24 atomic percent zinc; and 1 to 15 atomic percent aluminium. It will be understood that the alloys described herein may comprise incidental impurities. Preferably, the incidental impurities do not exceed 0.5 at. %, or preferably, 0.1 at. %, or more preferably, 0.05 at. %.

In certain examples, the present disclosure provides an alloy comprising or consisting of: 42.5 to 65 at. % Cu; 10 to 40 at. % Mn; 0.5 to 8 at. % Ni; 5 to 24 at. % Zn; and 1 to 5 at. % Al. In certain examples, the present disclosure provides an alloy comprising or consisting of: 44 to 64 at. % Cu; 8 to 40 at. % Mn; 1 to 8 at. % Ni; 6 to 20 at. % Zn; and 1 to 4 at. % Al. In certain examples, the present disclosure provides an alloy comprising or consisting of: 42 to 62.5 at. % Cu; 8 to 40 at. % Mn; 1 to 8 at. % Ni; 6 to 20 at. % Zn; and 1 to 4 at. % Al. In certain examples, the present disclosure provides an alloy comprising or consisting of: 42.5 to 65 at. % Cu; 8 to 40 at. % Mn; 1 to 5 at. % Ni; 6 to 20 at. % Zn; and 1 to 3 at. % Al. In certain examples, the present disclosure provides an alloy comprising or consisting of: 47.5 to 62.5 at. % Cu; 8 to 40 at. % Mn; 1 to 6 at. % Ni; 6 to 15 at. % Zn; and 1 to 3 at. % Al. In certain examples, the present disclosure provides an alloy comprising or consisting of: 47.5 to 65 at. % Cu; 8 to 40 at. % Mn; 1 to 6 at. % Ni; 6 to 13 at. % Zn; and 1 to 3 at. % Al. In certain examples, the present disclosure provides an alloy comprising or consisting of: 45 to 60 at. % Cu; 12.5 to 35 at. % Mn; 3 to 5 at. % Ni; 12.5 to 20 at. % Zn; and 2 to 3 at. % Al.

In certain examples, the present disclosure provides an alloy consisting of: about 60 at. % Cu; about 5 at. % Ni; about 15 at. % Mn; about 17.5 at. % Zn; and about 2.5 at. % Al. The present disclosure also provides an alloy consisting of: about 60 at. % Cu; about 5 at. % Ni; about 12.5 at. % Mn; about 20 at. % Zn; and about 2.5 at. % Al. The present disclosure also provides an alloy consisting of: about 57.5 at. % Cu; about 5 at. % Ni; about 15 at. % Mn; about 20 at. % Zn; and about 2.5 at. % Al. The present disclosure also provides an alloy consisting of: about 55 at. % Cu; about 5 at. % Ni; about 20 at. % Mn; about 17.5 at. % Zn; and about 2.5 at. % Al. The present disclosure also provides an alloy consisting of: about 55 at. % Cu; about 5 at. % Ni; about 17.5 at. % Zn; and about 2.5 at. % Al. The present disclosure also provides an alloy consisting of: about 57.5 at. % Cu; about 5 at. % Ni; about 15 at. % Mn; about 20 at. % Zn; and about 2.5 at. % Al. The present disclosure also provides an alloy consisting of: about 55 at. % Cu; about 5 at. % Ni; about 17.5 at. % Zn; and about 2.5 at. % Al.

% Mn; about 20 at. % Zn; and about 2.5 at. % Al. The present disclosure also provides an alloy consisting of: about 52.5 at. % Cu; about 5 at. % Ni; about 20 at. % Mn; about 20 at. % Zn; and about 2.5 at. % Al. The present disclosure also provides an alloy consisting of: about 52.5 at. % Cu; about 5 at. % Ni; about 22.5 at. % Mn; about 17.5 at. % Zn; and about 2.5 at. % Al. The present disclosure also provides an alloy consisting of: about 52.5 at. % Cu; about 5 at. % Ni; about 25 at. % Mn; about 15 at. % Zn; and about 2.5 at. % Al. The present disclosure also provides an alloy consisting of: about 52.5 at. % Cu; about 5 at. % Ni; about 27.5 at. % Mn; about 12.5 at. % Zn; and about 2.5 at. % Al. The present disclosure also provides an alloy consisting of: about 50 at. % Cu; about 5 at. % Ni; about 30 at. % Mn; about 12.5 at. % Zn; and about 2.5 at. % Al. The present disclosure also provides an alloy consisting of: about 50 at. % Cu; about 5 at. % Ni; about 27.5 at. % Mn; about 15 at. % Zn; and about 2.5 at. % Al. The present disclosure also provides an alloy consisting of: about 47.5 at. % Cu; about 5 at. % Ni; about 30 at. % Mn; about 15 at. % Zn; and about 2.5 at. % Al. The present disclosure also provides an alloy consisting of: about 47.5 at. % Cu; about 5 at. % Ni; about 32.5 at. % Mn; about 12.5 at. % Zn; and about 2.5 at. % Al. The present disclosure also provides an alloy consisting of: about 45 at. % Cu; about 5 at. % Ni; about 32.5 at. % Mn; about 15 at. % Zn; and about 2.5 at. % Al. The present disclosure also provides an alloy consisting of: about 45 at. % Cu; about 5 at. % Ni; about 35 at. % Mn; about 12.5 at. % Zn; and about 2.5 at. % Al. The present disclosure also provides an alloy consisting of: about 59 at. % Cu; about 3 at. % Ni; about 15.5 at. % Mn; about 20 at. % Zn; and about 2.5 at. % Al.

In some examples, the present disclosure provides an alloy comprising or consisting of: 5 to 40 at. % Mn; 1 to 24 at. % Ni; 5 to 24 at. % Zn; 1 to 15 at. % Al; and a balance of Cu. In some examples, the present disclosure provides an alloy comprising or consisting of: 8 to 40 at. % Mn; 1 to 8 at. % Ni; 5 to 24 at. % Zn; 1 to 15 at. % Al; and a balance of Cu. In some examples, the present disclosure provides an alloy comprising or consisting of: 8 to 40 at. % Mn; 1 to 8 at. % Ni; 5 to 24 at. % Zn; 1 to 5 at. % Al; and a balance of Cu. In some examples, the present disclosure provides an alloy comprising or consisting of: 12.5 to 35 at. % Mn; 1 to 7 at. % Ni; 7.5 to 24 at. % Zn; 1 to 5 at. % Al; and a balance of Cu. In some examples, the present disclosure provides an alloy comprising or consisting of: 12.5 to 35 at. % Mn; 1 to 7 at. % Ni; 7.5 to 20 at. % Zn; 1 to 5 at. % Al; and a balance of Cu. In some examples, the present disclosure provides an alloy comprising or consisting of: 22.5 to 35 at. % Mn; 1 to 5 at. % Ni; 7.5 to 12.5 at. % Zn; 1 to 3 at. % Al; and a balance of Cu. In some examples, the present disclosure provides an alloy comprising or consisting of: 17 to 35 at. % Mn; 1 to 8 at. % Ni; 9.5 to 20 at. % Zn; 0 to 5 at. % Al; and a balance of Cu. In some examples, the present disclosure provides an alloy comprising or consisting of: 17 to 35 at. % Mn; 1 to 8 at. % Ni; 9.5 to 20 at. % Zn; 1 to 5 at. % Al; and a balance of Cu. In some examples, the present disclosure provides an alloy comprising or consisting of: 17 to 35 at. % Mn; 1 to 8 at. % Ni; 9.5 to 15 at. % Zn; 1 to 5 at. % Al; and a balance of Cu. In some examples, the present disclosure provides an alloy comprising or consisting of: 17 to 35 at. % Mn; 1 to 8 at. % Ni; 9.5 to 12.5 at. % Zn; 1 to 5 at. % Al; and a balance of Cu. In some examples, the present disclosure provides an alloy comprising or consisting of: 17 to 35 at. % Mn; 1 to 8 at. % Ni; 9.5 to 12.5 at. % Zn; 1 to 3 at. % Al; and a balance of Cu. In some examples, the present disclosure provides an

alloy comprising or consisting of: 17 to 35 at. % Mn; 1 to 5 at. % Ni; 9.5 to 12.5 at. % Zn; 1 to 3 at. % Al; and a balance of Cu.

In some examples, the present disclosure provides an alloy comprising or consisting of: 40 to 62.5 atomic percent copper; 5 to 40 atomic percent manganese; up to 24 atomic percent nickel; 5 to 24 atomic percent zinc; 1 to 15 atomic percent aluminium; and up to 20 atomic percent of one or more elements selected from the group consisting of chromium, lead, bismuth, cobalt, iron, carbon, tin, silicon and magnesium. In some examples, the present disclosure provides an alloy comprising or consisting of: 40 to 62.5 atomic percent copper; 5 to 40 atomic percent manganese; up to 24 atomic percent nickel; 5 to 24 atomic percent zinc; 1 to 15 atomic percent aluminium; and up to 1 atomic percent of one or more elements selected from the group consisting of arsenic, phosphorus, sulphur and antimony. In some examples, the present disclosure provides an alloy comprising or consisting of: 40 to 62.5 atomic percent copper; 5 to 40 atomic percent manganese; up to 24 atomic percent nickel; 5 to 24 atomic percent zinc; 1 to 15 atomic percent aluminium; up to 20 atomic percent of one or more elements selected from the group consisting of chromium, lead, bismuth, cobalt, iron, carbon, tin, silicon and magnesium; and up to 1 atomic percent of one or more elements selected from the group consisting of arsenic, phosphorus, sulphur and antimony. It will be understood that in such examples, the alloy may comprise one or more of chromium, lead, bismuth, cobalt, iron, carbon, tin, silicon and magnesium, as long as the total concentration of the one or more elements does not exceed 20 at. %. Likewise, such alloys may comprise one or more of arsenic, phosphorus, sulphur and antimony, as long as the total concentration of the one or more elements does not exceed more than 1 at. %. In certain examples, arsenic, phosphorus, sulphur and antimony are present in an amount of about 0.5 at. % individually or about 0.7 at. % in total.

In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Cr. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Cr. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Bi. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Bi. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Fe. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Fe. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Sn. In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and up to 20 at. % Si. In some examples, the present disclosure provides an alloy comprising or consisting of 40 to 62.5 at. % Cu; 5 to

40 at. % Mn; up to 24 at. % Ni; 5 to 24 at. % Zn; 1 to 15 at. % Al; and up to 20 at. % Mg.

In some examples, the alloy comprises 0 to 7 at. % chromium, such as 0 to 5 at. % chromium, 0.5 to 4.5 at. % chromium, 0.5 to 4 at. % chromium, 0.5 to 3.5 at. % chromium, 1 to 3.5 at. % chromium, 1 to 3 at. % chromium, 1.5 to 3 at. % chromium or 1.5 to 2.5 at. % chromium. For example, the alloy may comprise about 0.5 at. %, about 0.75 at. %, about 1 at. %, about 1.25 at. %, about 1.5 at. %, about 1.75 at. %, about 2 at. %, about 2.25 at. %, about 2.5 at. %, about 2.75 at. %, about 3 at. %, about 3.25 at. %, about 3.5 at. %, about 3.75 at. %, about 4 at. %, about 4.25 at. %, about 4.5 at. %, about 4.75 at. %, about 5 at. %, about 5.25 at. %, about 5.5 at. %, about 5.75 at. %, about 6 at. %, about 6.25 at. %, about 6.5 at. %, about 6.75 at. % or about 7 at. % chromium. In some examples, chromium is not present in the alloy (ie, 0 at. %). In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and 0 to 7 at. % Cr, such as 0.5 to 5 at. % Cr.

In some examples, the alloy comprises 0 to 8 at. % lead, such as 0 to 6 at. % lead, 0.5 to 5.5 at. % lead, 0.5 to 5 at. % lead, 0.5 to 4.5 at. % lead, 1 to 4.5 at. % lead, 1 to 4 at. % lead, 1.5 to 3.5 at. % lead or 1.5 to 3 at. % lead. For example, the alloy may comprise about 0.5 at. %, about 0.75 at. %, about 1 at. %, about 1.25 at. %, about 1.5 at. %, about 1.75 at. %, about 2 at. %, about 2.25 at. %, about 2.5 at. %, about 2.75 at. %, about 3 at. %, about 3.25 at. %, about 3.5 at. %, about 3.75 at. %, about 4 at. %, about 4.25 at. %, about 4.5 at. %, about 4.75 at. %, about 5 at. %, about 5.25 at. %, about 5.5 at. %, about 5.75 at. %, about 6 at. %, about 6.25 at. %, about 6.5 at. %, about 6.75 at. %, about 7 at. %, about 7.25 at. %, about 7.5 at. %, about 7.75 at. % or about 8 at. % lead. In some examples, lead is not present in the alloy (ie, 0 at. %). In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and 0 to 8 at. % Pb, such as 0.5 to 6 at. % Pb.

In some examples, the alloy comprises 0 to 8 at. % bismuth, such as 0 to 5 at. % bismuth, 0.5 to 4.5 at. % bismuth, 0.5 to 4 at. % bismuth, 0.5 to 3.5 at. % bismuth, 1 to 3 at. % bismuth, 1 to 2.5 at. % bismuth or 1.5 to 2.5 at. % bismuth. For example, the alloy may comprise about 0.5 at. %, about 0.75 at. %, about 1 at. %, about 1.25 at. %, about 1.5 at. %, about 1.75 at. %, about 2 at. %, about 2.25 at. %, about 2.5 at. %, about 2.75 at. %, about 3 at. %, about 3.25 at. %, about 3.5 at. %, about 3.75 at. %, about 4 at. %, about 4.25 at. %, about 4.5 at. %, about 4.75 at. %, about 5 at. %, about 5.25 at. %, about 5.5 at. %, about 5.75 at. %, about 6 at. %, about 6.25 at. %, about 6.5 at. %, about 6.75 at. %, about 7 at. %, about 7.25 at. %, about 7.5 at. %, about 7.75 at. % or about 8 at. % bismuth. In some examples, the alloy comprises less than 0.7 at. % bismuth such as less than 0.5 at. % bismuth. In some examples, bismuth is not present in the alloy (ie, 0 at. %). In some examples, the present disclosure provides an alloy comprising or consisting of 40 to 62.5 at. % Cu; 5 to 40 at. % Mn; up to 24 at. % Ni; 5 to 24 at. % Zn; 1 to 15 at. % Al; and 0 to 8 at. % Bi, such as 0.2 to 2 at. % Bi, such as about 0.55 at. % or about 0.6 at. % Bi.

In some examples, the alloy comprises 0 to 8 at. % cobalt, such as 0 to 6 at. % cobalt, 0.5 to 5.5 at. % cobalt, 0.5 to 5 at. % cobalt, 0.5 to 4.5 at. % cobalt, 1 to 4.5 at. % cobalt, 1 to 4 at. % cobalt, 1.5 to 3.5 at. % cobalt or 1.5 to 3 at. % cobalt. For example, the alloy may comprise about 0.5 at. %, about 0.75 at. %, about 1 at. %, about 1.25 at. %, about 1.5

at %, about 1.75 at %, about 2 at %, about 2.25 at %, about 2.5 at %, about 2.75 at %, about 3 at %, about 3.25 at %, about 3.5 at %, about 3.75 at %, about 4 at %, about 4.25 at %, about 4.5 at %, about 4.75 at %, about 5 at %, about 5.25 at %, about 5.5 at %, about 5.75 at %, about 6 at %, about 6.25 at %, about 6.5 at %, about 6.75 at %, about 7 at %, about 7.25 at %, about 7.5 at %, about 7.75 at % or about 8 at % cobalt. In some examples, cobalt is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 8 at % Co, such as 0.5 to 5 at % Co.

In some examples, the alloy comprises 0 to 12 at % iron, such as 0 to 10 at % iron, 0.5 to 9 at % iron, 0.5 to 8 at % iron, 0.5 to 7 at % iron, 1 to 6.5 at % iron, 1 to 6 at % iron, 1.5 to 5.5 at % iron or 1.5 to 5 at % iron. For example, the alloy may comprise about 0.5 at %, about 0.75 at %, about 1 at %, about 1.25 at %, about 1.5 at %, about 1.75 at %, about 2 at %, about 2.25 at %, about 2.5 at %, about 2.75 at %, about 3 at %, about 3.25 at %, about 3.5 at %, about 3.75 at %, about 4 at %, about 4.25 at %, about 4.5 at %, about 4.75 at %, about 5 at %, about 5.25 at %, about 5.5 at %, about 5.75 at %, about 6 at %, about 6.25 at %, about 6.5 at %, about 6.75 at %, about 7 at %, about 7.25 at %, about 7.5 at %, about 7.75 at %, about 8 at %, about 8.25 at %, about 8.5 at %, about 8.75 at %, about 9 at %, about 9.25 at %, about 9.5 at %, about 9.75 at %, about 10 at %, about 10.25 at %, about 10.5 at %, about 10.75 at %, about 11 at %, about 11.25 at %, about 11.5 at %, about 11.75 at % or about 12 at % iron. In some examples, iron is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 12 at % Fe, such as 0.5 to 7 at % Fe.

In some examples, the alloy comprises 0 to 8 at % carbon, such as 0 to 6 at % carbon, 0.5 to 5.5 at % carbon, 1 to 5 at % carbon, 1.5 to 5 at % carbon, 1.5 to 5 at % carbon, 2 to 5 at % carbon, 2.5 to 5 at % carbon or 3 to 5 at % carbon. For example, the alloy may comprise about 0.5 at %, about 0.75 at %, about 1 at %, about 1.25 at %, about 1.5 at %, about 1.75 at %, about 2 at %, about 2.25 at %, about 2.5 at %, about 2.75 at %, about 3 at %, about 3.25 at %, about 3.5 at %, about 3.75 at %, about 4 at %, about 4.25 at %, about 4.5 at %, about 4.75 at %, about 5 at %, about 5.25 at %, about 5.5 at %, about 5.75 at %, about 6 at %, about 6.25 at %, about 6.5 at %, about 6.75 at %, about 7 at %, about 7.25 at %, about 7.5 at %, about 7.75 at % or about 8 at % carbon. In some examples, the alloy comprises less than 0.7 at % carbon such as less than 0.5 at % carbon. In some examples, carbon is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 8 at % C, such as 0.5 to 5 at % C.

In some examples, the alloy comprises 0 to 20 at % tin, such as 0 to 10 at % tin, 0.5 to 8 at % tin, 0.5 to 4 at % tin, 0.5 to 3.5 at % tin, 1 to 3 at % tin, 1 to 2.5 at % tin or 1.5 to 2.5 at % tin. For example, the alloy may comprise about 0.5 at %, about 0.75 at %, about 1 at %, about 1.25 at %, about 1.5 at %, about 1.75 at %, about 2 at %, about 2.25 at %, about 2.5 at %, about 2.75 at %, about 3 at %, about 3.25 at %, about 3.5 at %, about 3.75 at %, about 4 at %, about 4.25 at %, about 4.5 at %, about 4.75 at %, about 5 at %, about 5.25 at %, about 5.5 at %, about 5.75 at %, about 6 at %, about 6.25 at %, about 6.5 at %, about 6.75 at %, about 7 at %, about 7.25 at %, about 7.5 at %, about 7.75 at % or about 8 at % tin. In some examples, tin is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 20 at % Sn, such as 0.5 to 9 at % Sn.

In some examples, the alloy comprises 0 to 8 at % silicon, such as 0 to 6 at % silicon, 0.5 to 5.5 at % silicon, 0.5 to 5 at % silicon, 0.5 to 4.5 at % silicon, 1 to 4.5 at % silicon, 1 to 4 at % silicon, 1.5 to 3.5 at % silicon or 1.5 to 3 at % silicon. For example, the alloy may comprise about 0.5 at %, about 0.75 at %, about 1 at %, about 1.25 at %, about 1.5 at %, about 1.75 at %, about 2 at %, about 2.25 at %, about 2.5 at %, about 2.75 at %, about 3 at %, about 3.25 at %, about 3.5 at %, about 3.75 at %, about 4 at %, about 4.25 at %, about 4.5 at %, about 4.75 at %, about 5 at %, about 5.25 at %, about 5.5 at %, about 5.75 at %, about 6 at %, about 6.25 at %, about 6.5 at %, about 6.75 at %, about 7 at %, about 7.25 at %, about 7.5 at %, about 7.75 at % or about 8 at % silicon. In some examples, silicon is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 20 at % Si, such as 0.5 to 5 at % Si.

In some examples, the alloy comprises 0 to 2 at % magnesium, such as 0 to 1.75 at % magnesium, 0.25 to 1.75 at % magnesium, 0.25 to 1.5 at % magnesium or 0.5 to 1.5 at % magnesium. For example, the alloy may comprise about 0.25 at %, about 0.5 at %, about 0.75 at %, about 1 at %, about 1.25 at %, about 1.5 at %, about 1.75 at % or about 2 at % magnesium. In some examples, magnesium is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 8 at % Si, such as 0.5 to 5 at % Si.

In some examples, the alloy comprises 0 to 2 at % magnesium, such as 0 to 1.75 at % magnesium, 0.25 to 1.75 at % magnesium, 0.25 to 1.5 at % magnesium or 0.5 to 1.5 at % magnesium. For example, the alloy may comprise about 0.25 at %, about 0.5 at %, about 0.75 at %, about 1 at %, about 1.25 at %, about 1.5 at %, about 1.75 at % or about 2 at % magnesium. In some examples, magnesium is not present in the alloy (ie, 0 at %). In some examples, the present disclosure provides an alloy comprising or consisting of 40 to 62.5 at % Cu; 5 to 40 at % Mn; up to 24 at % Ni; 5 to 24 at % Zn; 1 to 15 at % Al; and 0 to 2 at % Mg, such as 0.2 to 1 at % Mg.

In some examples, the alloys of the present disclosure comprise up to 1 atomic percent of one or more elements selected from the group consisting of arsenic, phosphorus, sulphur and antimony. For example, an alloy of the present disclosure may comprise about 0.1 at %, about 0.2 at %, about 0.3 at %, about 0.4 at %, about 0.5 at %, about 0.6 at %, about 0.7 at %, about 0.8 at %, about 0.9 at % or about 1 at % As. In some examples, the alloy may comprise about 0.1 at %, about 0.2 at %, about 0.3 at %, about 0.4 at %, about 0.5 at %, about 0.6 at %, about 0.7 at %, about 0.8 at %, about 0.9 at % or about 1 at % P. In some examples, the alloy may comprise about 0.1 at %, about 0.2 at %, about 0.3 at %, about 0.4 at %, about 0.5 at %, about 0.6 at %, about 0.7 at %, about 0.8 at %, about 0.9 at % or about 1 at % S. In some examples, the alloy may comprise about 0.1 at %, about 0.2 at %, about 0.3 at %, about 0.4 at %, about 0.5 at %, about 0.6 at %, about 0.7 at %, about 0.8 at %, about 0.9 at % or about 1 at % Sb.

In some examples, the present disclosure provides an alloy comprising or consisting of: 40 to 62.5 atomic percent copper; 5 to 40 atomic percent manganese; up to 24 atomic percent nickel; 5 to 24 atomic percent zinc; 1 to 15 atomic percent aluminium; and up to 0.5 atomic percent carbon or bismuth. In some examples, the present disclosure provides an alloy comprising or consisting of: 45 to 62.5 atomic percent copper; 8 to 40 atomic percent manganese; 1 to 8 atomic percent nickel; 5 to 24 atomic percent zinc; 1 to 5

## 11

atomic percent aluminium; up to 0.4 atomic percent carbon; and up to 0.4 atomic percent bismuth.

Manganese, zinc and aluminium generally reduce the stacking fault energy of a copper alloy. Of these three elements, aluminium is the most potent, reducing the stacking fault energy at a rate of about  $3 \times \text{Zn}$ . Manganese provides a smaller decrease in stacking fault energy compared to zinc, generally about  $0.2 \times \text{Zn}$ . The alloys of the present disclosure preferably comprise manganese, zinc and aluminium in amounts that confer a stacking fault energy similar to that conferred by 22.5 to 35 at. % zinc. In certain examples, the alloys of the present disclosure comprise aluminium, zinc and manganese in the following amounts:

$$(3 \times \text{atomic percent of aluminium}) + \text{atomic percent of zinc} + (0.2 \times \text{atomic percent of manganese}) \text{ is between } 22.5\% \text{ and } 35\%.$$

Or, expressed differently:

$$[(3 \times \text{at. \% Al}) + (\text{at. \% Zn}) + (0.2 \times \text{at. \% Mn})] = 22.5 \text{ to } 35 \text{ at. \%}.$$

In some examples,  $(3 \times \text{atomic percent of aluminium}) + \text{atomic percent of zinc} + (0.2 \times \text{atomic percent of manganese})$  is between 22.5 at. % and 35 at. %, such as between 23.5 at. % and 32.5 at. %, between 24 at. % and 31 at. %, between 24.5 at. % and 30.5 at. %, between 25 at. % and 30 at. %, between 25.5 at. % and 29.5 at. %, between 26 at. % and 29.5 at. %, between 26.5 at. % and 29.5 at. %, or between 27 at. % and 29 at. %.

The ductility of a typical brass is largely a consequence of mechanical twinning within its microstructure. The ability of an alloy to twin is directly related to its stacking fault energy. An alloy with a low stacking fault energy generally twins more easily and is more ductile than an alloy with a high stacking fault energy. Increasing the nickel content of a copper alloy typically increases the alloy's stacking fault energy, thus increasing its strength but also decreasing its ductility. This can be less desirable for industry since the alloy requires more force to work it into shape. The alloys of the present disclosure preferably have more copper than nickel in atomic percent terms and are therefore more ductile and more easily worked compared to high-nickel alloys. For example, in the alloys of the present disclosure, the atomic percent ratio of copper:nickel may be at least 2, such as at least 3, or at least 4, at least 4.5, at least 5, at least 5.5, at least 6, at least 6.5, at least 7, at least 7.5, at least 8, at least 8.5, at least 9, at least 9.5, at least 10, at least 10.5, at least 11, at least 11.5, at least 12, at least 12.5, at least 13, at least 13.5, at least 14, at least 14.5, at least 15, at least 15.5, at least 16, at least 16.5, at least 17, at least 17.5, at least 18, at least 18.5, at least 19 or at least 19.5.

Copper is also known to be highly antimicrobial in a range of environments. Accordingly, the alloys of the present disclosure may be applied in situations where microbial resistance is desired. For example, the alloys described herein may be used in the manufacture of an autoclave, a door knob, cookware or a food container.

The alloys described herein are preferably low- or non-sparking, ie, they do not readily spark when they are struck mechanically, cut by metal tools or abraded/ground, thereby making them safe for use in volatile environments.

Although being present at lower levels compared to copper, the nickel in the present alloys may confer resistance to corrosion and increase the solubility of manganese and copper. Moreover, nickel may also hinder dezincification of the alloy in service. Dezincification occurs when zinc atoms

## 12

migrate to grain boundaries and to the surface, enriching these areas locally with zinc and causing localised corrosion and weakness in the alloy.

Microstructurally, certain alloys of the present disclosure may be predominantly single phase (alpha/face-centred-cubic crystal structure) or multi-phase, depending on constitution and applied heat treatment.

Certain alloys described herein may be hardenable via a crystal structure ordering mechanism or spinodal decomposition event when heat treated for long periods of time at moderate temperatures.

In certain examples, an alloy of the present disclosure has a tensile strain to failure of between about 25% and 70%, such as between about 30% and 65%, or between about 31% and 64%, or between about 35% and 65%, or between about 40% and 65%, or between about 45% and 65%, or between about 45% and 60%, or between about 50% and 65%, or between about 55% and 65% or between about 60% and 65%.

20 In certain examples, the alloy of the present disclosure has an ultimate tensile strength of between about 350 MPa and 600 MPa, such as between about 360 MPa and 600 MPa, or between about 370 MPa and 600 MPa, or between about 380 MPa and 600 MPa, or between about 380 MPa and 590 MPa, or between about 385 MPa and 590 MPa, or between about 390 MPa and 585 MPa, or between about 390 MPa and 580 MPa, or between about 390 MPa and 575 MPa, or between about 394 MPa and 572 MPa.

25 In some examples, the alloy of the present disclosure has an as-cast hardness ( $H_V$ ) of between about 70 and 190, such as between about 75 and 180, or between about 80 and 170, or between about 86 and 90, or between about 83 and 89, or between about 111 and 114, or between about 94 and 103, or between about 135 and 137, or between about 111 and 116, or between about 133 and 137, or between about 111 and 116, or between about 133 and 137, or between about 142 and 166, or between about 120 and 126, or between about 120 and 150, or between about 125 and 155, or between about 130 and 160, or between about 130 and 165, or between about 105 and 127, or between about 122 and 139, or between about 129 and 139, or between about 150 and 166, or between about 130 and 137, or between about 135 and 150, or between about 130 and 140, or between about 94 and 103.

30 The alloys of the present disclosure may be cast or pressure die-cast into a final product (casting alloys) at relatively low temperatures, hot forged, hot-rolled or hot-extruded into a plate or rod/tube, cold-rolled or cold forged into a plate rod or tube, deep-drawn, turned, milled or machined with metal cutting tooling to specification. The alloys may be soldered, brazed or welded. The alloys may also be chrome- or nickel-plated.

35 The alloys of the present disclosure may be used in general building fixtures and hardware, including door and window hinges, latches, door knobs, door locks, knockers, keys, decorative fixtures, as well as mobile phone casings, bezels, badges and medals, ornamental castings and statues.

The alloys may also be suitable for use in zippers, press 40 studs for clothing or baggage/luggage, gears, cogs, gear drive shafts, solid slip bearings, munitions/cartridge or shell cases, ammunition, marine/ship applications, air liquid/liquid/heating/cooling radiators, plumbing, currency, clamps, fasteners, nuts, bolts, screws, washers, acoustic devices such as speakers, resonators, tuning forks and musical instruments (eg, trumpet or trombone), electronic contacts, electrical conducting devices, circuitry electronic cou-

plings, hydraulic or pneumatic fluid transfer tubing couplings or connectors (high or low pressure), hydraulic or pneumatic manifolds, switches, gates and non-sparking tooling (eg, for use in explosive environments).

## EXAMPLES

Cu—Ni—Mn—Zn—Al alloy charge balances with a calculated final volume of 40 cm<sup>3</sup> were made from additions of near-pure copper, zinc and nickel. Manganese was added using a commercial 50/50 wt. % copper-manganese master alloy. Alloys were made in a two-step process:

1. Cu—Mn—Ni buttons were made in a Buhler electric arc melting furnace via cyclic melting of the copper and nickel balances with the copper-manganese master alloy. A titanium-gettered argon atmosphere was produced via purging of the melting chamber with high purity argon three times over and then evacuating using both roughing and turbo vacuum pumps to the order of 10<sup>-4</sup> mbar. The melting chamber was then filled to 60% of atmospheric pressure with high purity argon. This was followed by melting a titanium getter. Homogeneity of the Cu—Ni—Mn buttons was obtained via first melting of the nickel shot in direct contact with copper (thus allowing the copper to melt into the molten nickel). Repeated melting of the newly formed Cu—Ni alloy followed by melting of the Cu—Ni buttons into the Cu—Mn master alloy produced homogenous Cu—Ni—Mn buttons.
2. Production of the final alloy and the inclusion of zinc and aluminium was conducted using an induction furnace. The zinc and aluminium were placed at the bottom of a boron nitride-coated graphite crucible with the Cu—Ni—Mn buttons placed on top to minimise zinc evaporation. Melting of the complete Cu—Ni—Mn—Zn—Al charge balances was conducted in a circulating argon-rich environment inside the induction furnace chamber. Complete charge balances were melted twice in the induction furnace; this was found to aid with homogeneity. During the first alloying cycle, charge balances were heated to 1100° C. where they were held for two minutes to ensure complete melting of all charge components. Alloyed ingots were then left to cool in the crucible before being removed and mechanically cleaned/abraded to a lustrous finish, removing any oxide products. Ingots were inverted and

remelted in the induction furnace, again held at 1100° C. for two minutes, cooled to approximately 950° C., and the liquid metal poured (in air) into a 16 mm wide, 100 mm long, 50 mm deep copper mould.

- 5 The castings (100 mm×16 mm×35 mm) were sectioned into 50 mm×16 mm×35 mm blocks. One half of the casting was used for metallographic examination and hardness testing of the as-cast structure. The remaining half of the casting was processed via hot rolling and heat treatment. Initial heat treatment of the as-cast structures was conducted at 750° C. for two hours (with this heat treatment found to completely dissolve the as-cast microstructure in the Cu—Ni—Mn—Zn—Al alloys). Samples were then hot rolled at 750° C. in cross directions from a starting thickness of 16 mm down to 8 mm. The purpose of the hot rolling process was to close any casting pores or defects, consolidating the material, and to refine and recrystallise the grain structure, essentially reproducing industry processing. During the hot rolling process, samples were cyclically removed from a 750° C. furnace and rolled in 0.25 mm increments to their final thickness of 8 mm. Following the hot rolling process, samples received a final heat treatment of 750° C. for two hours to produce the final processed alloys in a hot rolled and annealed condition. At this stage, processed alloy billet had approximate dimensions of 8 mm×35 mm×90 mm. In order to produce tensile specimens from the processed alloy material, 8 mm×8 mm×62 mm strips were cut from the billet and machined into cylindrical tensile specimens with 4 mm gauge diameter and 20 mm gauge length in accordance with ASTM E8M. Tensile testing was conducted in accordance with ASTM A370 using an Instron tensile testing machine, laser extension meter and associated computer and data logger. Measured load and laser extension readings were recorded using software produced by Bluehill. Representative engineering stress-strain data are provided in FIGS. 1 and 2, and characteristic mechanical properties are set out in Table 1. Side profiles of alloys fractured under tension are shown in FIGS. 3 and 4.
- 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220

TABLE 1-continued

Compositions and characteristic mechanical properties of specific alloys (processed samples hot rolled at 750° C. and annealed at 750° C. for 2 hrs).

|                                                                                        | As-cast<br>hardness<br>(HV <sub>1</sub> ) | Processed<br>alloy<br>hardness<br>(HV <sub>1</sub> ) | 0.2%<br>Proof<br>Stress<br>(MPa) | Ultimate<br>Tensile<br>Strength<br>(MPa) | Tensile<br>Elongation<br>to Failure<br>(Strain %) |
|----------------------------------------------------------------------------------------|-------------------------------------------|------------------------------------------------------|----------------------------------|------------------------------------------|---------------------------------------------------|
| Cu <sub>45</sub> Ni <sub>5</sub> Mn <sub>32.5</sub> Zn <sub>15</sub> Al <sub>2.5</sub> | 135-150                                   | 137-144                                              | 253                              | 629                                      | 29                                                |
| Cu <sub>45</sub> Ni <sub>5</sub> Mn <sub>35</sub> Zn <sub>12.5</sub> Al <sub>2.5</sub> | 130-140                                   | 111-117                                              | 191                              | 519                                      | 47                                                |
| Cu <sub>59</sub> Ni <sub>3</sub> Mn <sub>15.5</sub> Zn <sub>20</sub> Al <sub>2.5</sub> | 94-103                                    | 85-95                                                | 155                              | 390                                      | 64                                                |

While the techniques described above in this example may be suitable for laboratory scale alloy production, those skilled in the art will understand that other methods may be used, particularly for industrial scale alloy production. For example, the alloys may be produced by large scale melting of all alloy constituents in an induction or resistance heated furnace until completely molten. This may include alloying higher melting-point constituents first while progressively lowering the melt temperature as lower melting-point constituents are added to avoid off-gassing of zinc and/or manganese. Additives, fluxes or coke may be used to reduce oxygen, hydrogen and other impurities in the melt and to protect the melt surface from further oxidation or degradation. The melt may then be cast as ingots. The ingots may then be cast or pressure die-cast directly into products. The alloy could also be continuously cast through a water-cooled graphite or copper or other metal nozzle in a fixed cross section to produce plate, bar, rod or hollow-section products. Alternatively, the melt may be twin-roll strip cast into sheet products. Products may be subsequently homogenised at temperatures above 700° C., hot rolled, hot-extruded, hot-drawn or forged to their required shape at temperatures above 600° C. Products may be cold-worked (rolled, extruded, forged or drawn) and tempered or hardened by low-temperature annealing.

Although the invention has been described with reference to specific embodiments, it will be appreciated by those skilled in the art that the invention may be embodied in many other forms.

The invention claimed is:

1. An alloy consisting of:  
about 60 to greater than about 50 atomic percent copper;  
about 15 to about 35 atomic percent manganese;  
about 1 to about 7 atomic percent nickel;  
about 7.5 to about 20 atomic percent zinc;  
about 1 to about 5 atomic percent aluminium; and  
incidental impurities

wherein (3× atomic percent of aluminium)+atomic percent of zinc+(0.2× atomic percent of manganese) is between about 23.5% and about 32.5%;

and wherein the alloy has ultimate strain of about 40-65%.

2. The alloy of claim 1 having about 15 to about 22.5 atomic percent manganese.

3. The alloy of claim 1 having about 15 to about 18.5 atomic percent manganese.

4. The alloy of claim 1 having about 17.5 to about 18.5 atomic percent manganese.

5. The alloy of claim 1 having about 1 to about 5 atomic percent nickel.

6. The alloy of claim 1 having about 15 to about 20 atomic percent zinc.

7. The alloy of claim 1 having about 1 to about 3 atomic percent aluminium.

8. The alloy of claim 1 having about 2 to about 3 atomic percent aluminium.

9. The alloy of claim 1 which is Cu<sub>57.5</sub>Ni<sub>5</sub>Mn<sub>17.5</sub>Zn<sub>17.5</sub>Al<sub>2.5</sub> or Cu<sub>55</sub>Ni<sub>5</sub>Mn<sub>17.5</sub>Zn<sub>20</sub>Al<sub>2.5</sub>.

10. The alloy of claim 1 having about 24.5 to about 35 atomic percent manganese.

11. The alloy of claim 10 having about 55 to greater than about 50 atomic percent copper.

12. The alloy of claim 10 having about 15 to about 20 atomic percent zinc.

13. The alloy of claim 10 having about 1 to about 3 atomic percent aluminium.

14. The alloy of claim 10 having about 2 to about 3 atomic percent aluminium.

15. The alloy of claim 10 which is Cu<sub>52.5</sub>Ni<sub>5</sub>Mn<sub>25</sub>Zn<sub>15</sub>Al<sub>2.5</sub>, Cu<sub>52.5</sub>Ni<sub>5</sub>Mn<sub>27.5</sub>Zn<sub>12.5</sub>Al<sub>2.5</sub>, Cu<sub>50</sub>Ni<sub>5</sub>Mn<sub>30</sub>Zn<sub>12.5</sub>Al<sub>2.5</sub>, Cu<sub>50</sub>Ni<sub>5</sub>Mn<sub>27.5</sub>Zn<sub>15</sub>Al<sub>2.5</sub>, Cu<sub>47.5</sub>Ni<sub>5</sub>Mn<sub>30</sub>Zn<sub>15</sub>Al<sub>2.5</sub>, Cu<sub>47.5</sub>Ni<sub>5</sub>Mn<sub>32.5</sub>Zn<sub>12.5</sub>Al<sub>2.5</sub>, Cu<sub>45</sub>Ni<sub>5</sub>Mn<sub>32.5</sub>Zn<sub>15</sub>Al<sub>2.5</sub>, or Cu<sub>45</sub>Ni<sub>5</sub>Mn<sub>35</sub>Zn<sub>12.5</sub>Al<sub>2.5</sub>.

16. The alloy of claim 1 which is Cu<sub>57.5</sub>Ni<sub>5</sub>Mn<sub>15</sub>Zn<sub>20</sub>Al<sub>2.5</sub> or Cu<sub>59</sub>Ni<sub>3</sub>Mn<sub>15.5</sub>Zn<sub>20</sub>Al<sub>2.5</sub>.

17. The alloy of claim 1 having an ultimate tensile strength of between about 350 MPa and about 600 MPa.

\* \* \* \* \*